

# United States Patent [19]

Arfaei et al.

[11] Patent Number: 4,656,115

[45] Date of Patent: Apr. 7, 1987

[54] **EMULSION POLYMERIZATION OF METHACRYLONITRILE IN THE PRESENCE OF A CATIONIC EMULSIFIER AS A VEHICLE FOR VESICULAR PHOTOGRAPHY**

[75] Inventors: Ahmad Arfaei, Holyoke; Everett W. Bennett, Longmeadow, both of Mass.

[73] Assignee: James River Graphics, Inc., South Hadley, Mass.

[21] Appl. No.: 800,108

[22] Filed: Nov. 22, 1985

## Related U.S. Application Data

[63] Continuation of Ser. No. 474,057, Mar. 10, 1983, abandoned.

[51] Int. Cl.<sup>4</sup> ..... G03C 1/52; G03C 1/60

[52] U.S. Cl. ..... 430/170; 430/152; 430/176; 430/192; 430/197; 430/270; 430/290

[58] Field of Search ..... 430/152, 176, 197, 192, 430/290, 170, 270

| [56]                  | References Cited                     |
|-----------------------|--------------------------------------|
| U.S. PATENT DOCUMENTS |                                      |
| 3,161,511             | 12/1964 Parker et al. .... 430/152   |
| 3,457,071             | 7/1969 Notley et al. .... 430/152    |
| 3,622,333             | 11/1971 Cope .... 430/152            |
| 3,622,335             | 11/1971 Notley .... 430/152          |
| 3,622,336             | 11/1971 Notley .... 430/152          |
| 3,661,589             | 5/1972 Notley .... 430/152           |
| 4,215,191             | 7/1980 Kwok .... 430/152             |
| 4,219,616             | 8/1980 Pope et al. .... 430/152      |
| 4,272,603             | 6/1981 Chenevert et al. .... 430/152 |

*Primary Examiner*—Charles L. Bowers, Jr.  
*Attorney, Agent, or Firm*—Burns, Doane, Swecker & Mathis

## [57] ABSTRACT

An improved vesicular matrix prepared by the emulsion polymerization of methacrylonitrile, either alone or with a small amount of comonomer, in the presence of a cationic emulsifier. The resulting polymer or copolymer can be used alone, or the polymer or copolymer may be blended with a small amount of a highly incompatible polymer or copolymer, to provide an improved vesicular matrix.

3 Claims, No Drawings

EMULSION POLYMERIZATION OF  
METHACRYLONITRILE IN THE PRESENCE OF A  
CATIONIC EMULSIFIER AS A VEHICLE FOR  
VESICULAR PHOTOGRAPHY

This application is a continuation of application Ser. No. 474,057, filed Mar. 10, 1983, now abandoned.

BACKGROUND OF THE INVENTION

1. Field of the Invention

The present invention relates to vesicular photography, and more particularly, to improved vesicular matrices for use in vesicular photography, including novel polymers and copolymers useful therein.

2. Description of the Prior Art

Diazo type photoreproduction is of two different types. Each is based on the light sensitivity of aromatic diazo salts and the fact that such salts undergo two different types of reactions: (1) decomposition, in which nitrogen is lost or evolves as nitrogen gas and some other atom or group attaches to the benzene ring in its stead; and (2) "coupling", wherein the nitrogen of the diazo function is retained and the salts react with certain couplable color-forming components, i.e., a "coupler" or "azo-coupling component", to effect formation of an azo dye species.

The present invention, a vesicular process, is concerned with the former type of reaction. Vesicular images are formed in a photographic film by small bubbles or vesicles of gas which are formed and trapped in the areas of the film exposed to light and which refract light. Vesicular film consists of a colloidal or a resin coating or vehicle on a backing material and a light sensitive agent or sensitizer, such as a diazo compound, dispersed throughout the coating. When the film is exposed to light, the sensitizer releases molecules of a gas. In the case of diazo compounds, the gas is nitrogen. Rather than forming vesicles immediately, the vesicles are formed when the film is heated, presumably because the vehicle is relaxed sufficiently on heating for the gas molecules to form bubbles, and for the bubbles to expand. The formation of the vesicles makes the vehicle opaque to transmission of light in the exposed areas, resulting in the reflection and scattering of light from the vesicles.

Preservation of the image depends upon the vehicle maintaining its rigidity and the vesicles being fixed in place. Although the rigidity of the vehicle is reduced during development to permit gas molecules to diffuse together to form the vesicles and to allow the vesicles to expand, the rigidity is restored by cooling to give permanency to the image after development. For permanency, the vehicle must remain rigid under the heat and moisture conditions to which it will be exposed.

The first vesicular materials employed gelatin as the vehicle. However, such images faded rapidly because of the sensitivity of gelatin to water. Gelatin vehicles absorb moisture from the atmosphere and become soft, allowing the vesicle to collapse, thereby destroying the image.

Numerous patents describe later attempts at developing vesicular matrices. Although numerous such matrices have been developed, only three systems are currently being employed commercially; those being systems based on Saran, polyhydroxyethers of phenols, and poly-alpha-chloroacrylonitrile.

One material which appeared promising but has never been commercialized is polymethacrylonitrile. Despite a suitable softening point and a suitably low diffusion constant for nitrogen, its potential has yet to be realized.

The basic patent concerning polymethacrylonitrile is U.S. Pat. No. 3,161,511 to Parker and Mokler which describes a vehicle manufactured using polymethacrylonitrile as the resin matrix. As stated in that patent, homopolymers are preferable to copolymers because they are easier to manufacture.

The difficulty in the manufacture of copolymers is controlling proportions when there are two or more monomers. Monomers typically do not polymerize at

15 the same rate, i.e. if two monomers are polymerized together, one will enter into the reaction more easily than the other. As the reaction proceeds, the more reactive monomer will be consumed more rapidly, and the relative proportions of the two monomers will change.

20 Since the rate at which the monomers enter into the reaction depends on their relative proportions as well as their inherent activity toward the reaction, their reaction rates change. As the reaction proceeds, the relative proportion of the monomers entering the growing polymer changes, and the polymer produced at the beginning of the reaction has different monomer proportions from the polymer produced later.

To avoid this result, at least in part, monomer is sometimes continuously added during the reaction to maintain constant proportions. Another possibility is to accept variations in the proportions of the monomers in the polymer and to later thoroughly blend the resulting polymers to assure uniform properties throughout each batch. The average properties then meet the needs of 35 the product. However, this may result in variations from batch to batch because of variations in the completeness of the reaction or other conditions.

U.S. Pat. Nos. 3,622,335 and 3,622,336 to Notley are improvements on the Parker and Mokler patent mentioned above. These patents represent attempts to produce copolymers in spite of the problems discussed in the Parker and Mokler patent. The '335 patent employs copolymers of alpha substituted acrylonitrile (which includes methacrylonitrile) and a styrene-type monomer. It is stated therein that the proportion of comonomer must exceed 5 mole percent, and it is not generally desired to exceed 60 mole percent or the desired characteristics of the substituted acrylonitrile will not be obtained. Furthermore, it is stated that any two copolymers produced therein can be blended where they are compatible in a common solvent or mixed solvent, and that the essential polymer can be blended with limited amounts of a non-essential but compatible polymer such as cellulose acetate, cellulose acetate butyrate, polyaliphatic styrene, polyvinylidene chloride, acrylonitrile copolymer and polymethylmethacrylate.

The '336 patent is similar to the '335 patent except that it describes a copolymer of alpha-chloroacrylonitrile and alpha-methacrylonitrile. The ratio of the monomers was stated to be between 1:4 and 4:1, and a preferred ratio was stated to be 1:2.

U.S. Pat. No. 3,661,589 to Notley describes a different approach. Rather than copolymerization, a vesicular imaging film was formed by mutually dispersing two 65 resin solutions at the threshold of compatibility but having a common or mutual solvent, each of the resin solutions containing a sensitizer which liberates gas on irradiation, coating the resulting dispersion as a thin

film, and then drying. The resulting thermoplastic film is stated to be an intimate dispersion of one hydrophobic resin in the other hydrophobic resin with the sensitizer dispersed throughout.

The Notley '589 patent also sets forth the criteria that a hydrophobic resin used in vesicular photography must satisfy, and reiterates that these criteria are very comprehensive and quite critical. These include very low permeability, good rigidity under ambient conditions, a convenient softening temperature at which the polymer is sufficiently fluid to permit vesicles to form but at which the gas permeability is still not excessively high, good solubility, good film forming characteristics, good adhesion to inert substrates and good tolerance for high concentrations of sensitizer.

In the structure described in the Notley '589 patent, hydrophobic resin is encapsulated within a continuous coating of another hydrophobic resin, with the light sensitive gas generating material dispersed throughout the encapsulated and the encapsulating resin. The optimum amount of encapsulated resin is stated to exceed 5% but generally not to exceed 50% of the total resin. The threshold incompatibility described therein is illustrated by mixing two parts of a 20% solution of polystyrene in butanone with one part of a 20% solution of a polyvinylidene chloride/acrylonitrile copolymer in the same solvent. By using polystyrene to Saran in a ratio between 1 to 1 and 1 to 6, the solution is only slightly hazy and good coating quality is said to be achieved from the agitated solution. The threshold incompatibility is seen when the dispersion is allowed to stand since it separates into two layers, one rich in polystyrene and the other in Saran. Preferred encapsulating resins therein are Saran, polyvinyl acetals, copolymers of methacrylonitrile, and chloroacrylonitrile homopolymer and copolymers. The choice of encapsulated resin is based on the diffusion coefficient and the refractive index. Encapsulating/encapsulated resin combinations listed include Saran with polystyrene, ortho/para poly-chlorostyrene or cellulose acetate; polyvinyl formal with polystyrene or cellulose acetate; polyvinyl formal with polystyrene or polyketone; methacrylonitrile-methylmethacrylate copolymer with Saran or cellulose acetate; and chloroacrylonitrile-styrene copolymer with polystyrene.

While polymethacrylonitrile has a suitable softening point ( $T_g = 120^\circ C$ ) which should supply good developing and good thermal stability of vesicles, and has a diffusion coefficient for nitrogen which is also very low (approximately  $5 \times 10^{-13}$ ) which should prevent nitrogen from escaping prior to the development of the film, the technology described by the above patents is not currently being used commercially. Such compositions are slow in comparison to presently marketed films, with the problem appearing to be related to insufficient nucleation, possibly because of high lattice homogeneity of the polymer. For example, in comparison to a similar polymer (poly-alpha-chloroacrylonitrile), a polymethacrylonitrile film is much slower.

Accordingly, a need exists for a vesicular vehicle having the desirable properties of polymethacrylonitrile with a speed comparable to those of commercially available materials.

#### SUMMARY OF THE INVENTION

One object of the present invention is the provision of a polymer of methacrylonitrile prepared by emulsion polymerization in the presence of a cationic emulsifier.

Another object of the present invention is the provision of a copolymer of methacrylonitrile and less than 5 wt. % of a second monomer, a homopolymer of the second monomer being a polymer which would be incompatible with polymethacrylonitrile, the copolymer being prepared by emulsion polymerization in the presence of a cationic emulsifier.

Yet another object of the invention is the use of the polymer and/or the copolymer as the continuous phase of a light sensitive vesicular material.

Still another object of the invention is the use of the polymer and/or the copolymer blended with less than 5% of a second polymer or copolymer as the continuous phase of a light sensitive vesicular material.

#### DETAILED DESCRIPTION OF THE INVENTION

As stated above, the present invention comprises in one embodiment, homopolymer and copolymers of methacrylonitrile prepared by emulsion polymerization in the presence of a cationic emulsifier.

The polymethacrylonitrile of the present invention differs from the prior art in that it is produced by emulsion polymerization in the presence of cationic emulsifiers, whereas the polymethacrylonitrile of the prior art was produced by using anionic or nonionic emulsifiers. The use of cationic emulsifiers provides a novel polymethacrylonitrile which is particularly useful as a vesicular matrix. This is in contrast to the generally held belief in the prior art that emulsion polymerization using cationic emulsifiers was not commercially important because it was slower and gave inferior results.

As stated above, an alternative embodiment of the present invention constitutes copolymers of methacrylonitrile with other monomers, the homopolymers of which would be incompatible with polymethacrylonitrile, prepared by emulsion polymerization in the presence of a cationic emulsifier. An example of a suitable comonomer is methacrylamidopropyltrimethyl ammonium chloride, a cationic water soluble monomer. Other suitable comonomers include vinyl acetate, vinyl propionate, and other similar monomers. When used as a comonomer at a weight ratio of 1:20 or less to the methacrylonitrile, copolymers having excellent photospeed are produced.

Although any cationic emulsifier can be used in preparing the polymers and copolymers of the present invention, the following have been found to provide particularly good results: Adogen 432 (trademark of Sherex Chemical Co., Inc. for dialkyl ( $C_{12}-C_{18}$ ) dimethyl ammonium chloride); Lodyne S-106 (trademark of Ciba-Geigy for fluoroalkylammonium chloride); Ethoquad C/25 (trademark of Armour Industrial Chemicals Co. for methylpolyoxyethylene ( $C_{15}$ ) cocoammonium chloride); Barquat CME-35 (trademark of Lonza, Inc. for N-cetyl-N-ethyl-morpholinium chloride); and Uniquad CB-50 (trademark of Lonza, Inc. for 1-hydroxyethyl-1-benzyl 2-alkyl imidazolinium chloride).

The amount of emulsifier used can vary over a wide range from about 0.5% to about 10% by weight. The amount of emulsifier used will vary depending upon the ability of the particular emulsifier to stabilize the emulsion.

The use of cationic emulsifiers is preferably combined in the present invention with the use of radial initiators such as azobisisobutyronitrile; 2,2'-azobis(2,4-dimethylpentane nitrile); or 2,2-azobis(2,4-dimethyl-4-methoxy-

pentane nitrile). Other organic and inorganic initiators can also be used in the practice of the present invention including various peroxides and persulfates such as potassium persulfate. Such initiators are used in the present invention at an effective initiating concentration, typically between about 0.3 and about 5% w/w of monomer, preferably about 1-3%, and more preferably about 1-1.5%.

If desired, chain transfer agents can also be employed in the practice of the present invention. Various such agents, such as various mercaptans, are well known to those skilled in the art. A preferred chain transfer agent is dodecyl mercaptan.

While not wishing to be bound by theory, it is believed that the beneficial properties of the polymers and copolymers of the present invention are related to their molecular weight range and distribution which appear to depend somewhat on the amount of initiator employed. The preferred viscosity average molecular weight ( $M_v$ ) for the present invention is between about 10,000 and about 600,000, and more preferably between about 100,000 and about 300,000.

One indication that molecular weight is a relevant factor is the polydispersity of the polymers and copolymers of the present invention. Polydispersity is a measure of the range of different molecular weights in a sample. Polydispersity is typically stated as a ratio of the weight average molecular weight ( $M_w$ ) to the number average molecular weight ( $M_n$ ).  $M_n$  is essentially the ratio of the weight of the molecules to the total number of molecules. In contrast,  $M_w$  is a weighted average such that the larger the size of a molecule, the greater its contribution to  $M_w$ . Since polymerizations always results in a range of molecular weights,  $M_w$  will always be greater than  $M_n$ . Thus, the polydispersity ratio will always be greater than one. A typical polydispersity ratio for an emulsion polymerization is about 2.5:1. In contrast, the polydispersity ratio of the polymers of the present invention are high, typically above about 5:1, and preferably between about 6:1 and 11:1. Accordingly, it seems likely that not only the viscosity average molecular weight, but also the molecular weight distribution is important for optimizing the properties of the resulting polymer.

For the polymers and copolymers of the present invention,  $M_w$  is preferably between about 50,000 and about 1,500,000, and  $M_n$  is preferably between about 10,000 and about 300,000.  $M_w$  and  $M_n$  are readily determined by methods well known to those skilled in the art, one such method being gel permeation chromatography.

Another alternative embodiment of the present invention is the blending of methacrylonitrile polymer or copolymer produced according to the present invention with other polymers or copolymers. Examples of such polymers are polyvinyl acetate and copolymers of vinyl acetate and vinyl chloride. Such polymers or copolymers are typically used in small amounts, e.g. less than about 5% by weight, preferably less than about 3% by weight.

This embodiment of the present invention should be distinguished from blending of larger amounts (40-90%) of other resins to improve the photospeed of the blend such as that described in U.S. Pat. No. 4,272,603 to Chenevert et al. The system described therein utilizes polymethacrylonitrile at moderate molecular weights. Incorporation of 40 to 90% of an incompatible resin is possible only when the polymeth-

acrylonitrile has a very low molecular weight (less than about 10,000). While that patent does not directly mention the molecular weight of the polymethacrylonitrile used in the Examples, the molecular weight can be derived from the described properties which were improved with blending. Reference should also be made to column 3, lines 55-61 of Chenevert et al wherein it is stated that it is preferable to use lower molecular weight polymers of methacrylonitrile because they are compatible with other polymers over a wider range of proportions, and further that particularly useful polymers have a weight average size of 1440 to 2450.

In preparing films, it is preferred that the composition also contain a nucleating agent. Various nucleating agents are well known in the prior art. Particularly suitable for use in the present invention are anionic, cationic and nonionic fluorocarbon surfactants. Nucleating agents are typically added in small amounts, typically between about 0.02% and about 2.0% by weight, preferably between about 0.1 and about 1.0% by weight.

The vesiculating agent employed in preparing the vesicular film is sensitive to radiation, e.g., light, so that exposure to the radiation causes decomposition and formation of gas vesicles, preferably of nitrogen. Examples of suitable vesiculating agents include the following:

- 30 p-diazo-diphenylamine sulfate;
  - p-diazo-dimethylaniline zinc chloride;
  - p-diazo-diethylaniline zinc chloride;
  - p-diazo-ethyl-hydroxyethylaniline . one-half zinc chloride;
  - 35 p-diazo-methyl hydroxyethylaniline . one-half zinc chloride;
  - p-diazo-2,5-diethoxy-benzoylaniline . one-half zinc chloride;
  - p-diazo-ethyl-benzylaniline . one-half zinc chloride;
  - 40 p-diazo-dimethylaniline borofluoride;
  - p-diazo-2,5-dibutoxy-benzoylaniline . one-half zinc chloride;
  - p-diazo-1-morpholino benzene . one-half zinc chloride;
  - p-diazo-2,5-dimethoxy-1-p-tolyl-mercapto benzene . one-half zinc chloride;
  - p-diazo-3-ethoxy-diethylaniline . one-half zinc chloride;
  - p-diazo-2,5-diisopropoxy-1-morpholino benzene sulfosalicylate;
  - 50 p-diazo-2,5-diisopropoxy-1-morpholino benzene triflate;
  - p-diazo-2,5-diethoxy-1-morpholino benzene sulfosalicylate;
  - p-diazo-2,5-diethoxy-1-morpholino benzene triflate;
  - 55 2,5,4'-triethoxy-diphenyl-4-diazonium oxalate;
  - p-diazo-diethylaniline . one-half chloride;
  - p-diazo-2,5-dibutoxy-1-morpholino-benzene chloride . zinc chloride;
  - p-diazo-2,5-dimethoxy-1-morpholino-benzene chloride . zinc chloride;
  - p-diazo-2,5-diethoxy-1-morpholino-benzene chloride . one-half zinc chloride;
  - 60 2-diazo-1-naphthol-5-sulfonic acid;
  - p-diazo-diethylaniline borofluoride;
  - p-diazo-2-chloro-diethylaniline . one-half zinc chloride.
- Other suitable light-sensitive, nitrogen-forming compounds are the quinone-diazides, e.g.,



and azide compounds of the type



Also the carbazido (carboxylic acid azide) compounds containing a hydroxyl or amino-group in the position ortho to the carbazine group as described in U.S. Pat. No. 3,143,418 would be useful.

It is to be understood that the various physical characteristics of the polymeric materials employed in the present vesicular film system can be varied as desired by the addition of modifiers. Moreover, various materials can be added for the preservation of the sensitizer compound employed, e.g., various acids as taught in the art. Moreover, other materials, such as dyes and other compounds, can be added to improve the photometrics of a particular film without departing from the true scope and spirit of the present invention.

Where a support is employed on which the present vesicular photographic material is overcoated, the support can be any suitable material which is compatible with the medium, e.g. glass, polymeric materials, paper and the like. A polyethylene terephthalate base material is preferred since it has excellent chemical and physical stability under standard processing conditions and it has excellent dimensional stability. As is well known in the art, where a transparent support is employed a vesicular image recorded thereon in the conventional manner produces a corresponding image having the opposite photographic sign. However, the use of an opaque support, e.g. a black support, will produce a photographic image having the same photographic sign.

The vehicle and the sensitizer may be combined by any suitable method. However, it is preferred that they each be dissolved in a solvent and the resultant solutions combined. In this embodiment it is only necessary that the respective solutions be mutually miscible. For the most part, solvents such as alcohols, ketones, nitriles, esters, ethers and halogenated solvents may be used. Particularly useful are methyl, ethyl and isopropyl alcohols, alkyl acetates, acetone, methyl ethyl ketone, dioxane and acetonitrile. However, any inert solvent which meets the above miscibility requirement may be used.

If a diazo compound is used, as is preferred, it is generally dissolved in a small quantity of a polar solvent such as methanol, aqueous methanol, acetonitrile or acetone, and then added dropwise to the stirred resin solution to minimize precipitation of either the salt or the polymer. The preferred amount of the diazo compound is about 4 to 10 percent by weight of the resin used.

When a diazo compound is used as the vesiculating agent, it is preferred, but not necessary, that the solvent in which the diazo compound is dissolved be compatible with the solvent system selected for the resin in

order to minimize the possibility of the diazo compound or the resin precipitating out when the two solutions are mixed. It is understood in the art that a uniform dispersion of the vesiculating agent in the vehicle is desired.

After the film is thus prepared, there are at least three different methods of processing it. In one form, the film is exposed to image forming light, e.g., by being placed in contact with a transparency and exposed to light passing through the transparency, then the film is heated to 160°-300° F., for 1/10 to 3 seconds. This will produce an image of the opposite photographic sign from the transparency. Thus, if the transparency is negative, a positive vesicular photograph will result.

A second processing system which can be used is that described in U.S. Pat. No. 2,911,299. In it, the film is exposed to image forming light and gas released by the sensitizer is allowed to diffuse from the vehicle at a temperature too low for development to take place. Then the film is exposed overall to uniform light which actuates non-decomposed sensitizer, and it is heated to cause development at 160°-300° F. for 1/10 to 3 seconds either during or shortly after the second exposure, but before the gas has substantially diffused from the film. This results in image formation in areas not originally struck by light and an image of the same photographic sign as the transparency.

The third processing system is that described in U.S. Pat. No. 3,457,071. In that system, the film is exposed to image forming light of relatively low intensity for at least about 0.5 second and preferably for at least about 2.0 seconds. That is, the light is of low enough intensity that the film does not receive a normal exposure in less than 0.5 second and preferably 2.0 seconds. Then the film receives an overall exposure of light intensity which is sufficient to expose the film in less than 0.2 second and preferably less than 0.01 second. Overexposure or longer exposure can be tolerated, but there must be sufficient light to properly expose the film during the indicated time. This procedure avoids a separate diffusion step as used in the method of U.S. Pat. No. 2,911,299. In some cases, no heating is required to cause development, and the image appears spontaneously. However, in other cases, some heating may be used to advantage, as more fully described in U.S. Pat. No. 3,457,071.

In order to further illustrate the present invention and the advantage thereof, the following specific examples are given, it being understood that they are intended only to be illustrative without limiting the scope of the present invention.

#### EXAMPLE I

To a one liter flask was added 400 ml of deaerated tap water. To this was added 7.0 g of Adogen 432 (trademark of Sherex Chemical Co., Inc. for dialkyl (C<sub>12</sub>-C<sub>18</sub>) dimethyl ammonium chloride which is 67-69% pure) and 2.0 g of Lodyne S106 (trademark of Ciba-Geigy for fluoroalkyl ammonium chloride) which were dissolved with gentle stirring. Next 100.0 g of distilled methacrylonitrile was added and the contents heated to 69°-70° C. (The distillation was for the removal of any inhibitor.) Stirring was continued while 3.0 g of azobisisobutyronitrile was added. The reaction was allowed to proceed for 8.6 hours after which the contents of the flask were cooled to room temperature and then coagulated from emulsion by the addition of a saturated solution of sodium chloride. The polymer was washed with

several aliquots of methanol to ensure that no surfactant remained. The polymer was then dried at 81° C. for 48 hours before measurements were made or incorporation into a film coating. The resulting polymer had a  $M_v$  of 42,587, a  $M_n$  of 39,200 and a  $M_w$  of 292,000, giving the polymer a polydispersity ratio of 7.43:1.

To prepare a film coating, 10.0 g of the polymer was dissolved in 36.0 g of methyl ethyl ketone and 4.0 g of ethylene glycol monomethyl ether. To this was added a second solution containing 2.5 g of 1 wt. % Lodyne S-107 (trademark of Ciba Geigy for fluoroalkyl polyoxyethylene, a nonionic surfactant) in methyl ethyl ketone, and 0.25 g of 10 wt. % polyvinyl acetate in methyl ethyl ketone, 8.0 g of 1 wt. % Orasol Brilliant Blue G-N (trademark of Ciba-Geigy for a blue dyestuff) in methyl ethyl ketone, and 0.8 g of 3,6-diethoxy-4-morpholino-benzene diazonium tetrafluoroborate. The resulting solution was filtered and then coated onto a

II, it possessed a speed of 158.5% compared to commercially available Xidex SX Film.

#### EXAMPLES IV-VIII

To illustrate the dependence of photospeed on viscosity average molecular weight and polydispersity and how the initiator varies same, Example I was repeated with varying amounts of azobisisobutyronitrile. For each example, 100 g of methacrylonitrile, 7 g of Adogen 432 (trademark of Sherex Chemical Co., Inc. for dialkyl ( $C_{12}-C_{18}$ ) dimethyl ammonium chloride) and 2 g of Lodyne S-106 (trademark of Ciba-Geigy for fluoroalkylammonium chloride) were used, the latter two ingredients being the cationic emulsifiers used as received as solutions. For each example, the reaction temperature was 69°-70° C. and the speed of the resulting film was compared with Xidex SX film. The results are given in Table I.

TABLE I

| Example | Initiator (grams) | Water (ml) | Reaction Time (Hours) | Yield (%) | $M_v$   | $M_w$     | $M_n$   | $M_w/M_n$ | Photo-Speed |
|---------|-------------------|------------|-----------------------|-----------|---------|-----------|---------|-----------|-------------|
| IV      | 0.5               | 405        | 10.05                 | 93.67     | 544,848 | —         | —       | —         | 89.12       |
| V       | 3.0               | 404        | 9.02                  | 94.06     | 56,256  | 488,000   | 72,600  | 6.71      | 134.9       |
| VI      | 3.0               | 402        | 8.60                  | 100.00    | 39,153  | —         | —       | —         | 154.9       |
| VII     | 1.0               | 403        | 10.3                  | 93.61     | 189,084 | 1,240,000 | 144,000 | 8.63      | 97.7        |
| VIII    | 2.0               | 403        | 9.50                  | 98.88     | —       | 603,000   | 78,700  | 7.65      | 144.5       |

polyester film having a suitable bonding layer using a No. 22 Mayer Rod. After coating, the film was allowed to dry for one minute at room temperature and for two minutes in an oven maintained at 240° F. The film was processed using a Kodak #2 Photographic Step Tablet as a master. The film was exposed and developed in a commercially available A/M Bruning OP-57 Processor.

The photospeed was compared to commercially available Xidex SX Film developed in the same manner, with the result that the film prepared with the above polymer had a photospeed which was about 47.9% faster than the Xidex SX Film.

#### EXAMPLE II

Example I was repeated except that 5 g of a 50 wt. % solution of methacrylamidopropyltrimethyl ammonium chloride in water were used with 95 g of methacrylonitrile instead of solely methacrylonitrile monomer, and only 2.4 g of Adogen 432 (trademark of Sherex Chemical Co., Inc. for dialkyl ( $C_{12}-C_{18}$ ) dimethyl ammonium chloride) were used. The yield was 77.98% by weight.

A film was prepared and exposed as in Example I except that the polymer was blended with 0.25 g of polyvinylacetate as a 10% solution in methyl ethyl ketone. The resulting film had 129% of the photospeed of Xidex SX Film. Film was also processed in an A/M Bruning OP-57 Processor and found to possess 190.5% of the photospeed of Xidex SX Film.

#### EXAMPLE III

Example I was repeated except that 3 g of potassium persulfate were used instead of azobisisobutyronitrile, only 1.2 g of Adogen 432 were used, 408 ml of water were used, and the reaction time was 16 hours. The reaction yielded 81% of the polymer having a  $M_v$  of 103,672.

When used to prepare a film and processed as in Example I, the resulting film had a speed of 147.9% compared to commercially available Xidex SX Film. When a film was prepared and processed as in Example

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070

the presence of a cationic emulsifier or the copolymer of (a) with a photospeed-enhancing amount less than 5 weight percent of a polymer or copolymer of vinyl acetate which would be incompatible with said polymer or copolymer of methacrylonitrile; and

an effective gas-producing amount of a photosensitive solid agent substantially uniformly dispersed within said coating, which agent is capable of decomposing to produce nitrogen gas upon exposure to light.

3. A light sensitive vesicular material comprising a film support and a coating thereon, the continuous phase of said coating comprising:

(a) a copolymer of methacrylonitrile and a photospeed-enhancing amount less than 5 weight percent of a second monomer which is a cationic water soluble monomer or a vinyl ester, a homopolymer of the second monomer being a polymer which

20

would be incompatible with polymethacrylonitrile, said copolymer being prepared by emulsion polymerization in the presence of a cationic surfactant, or

(b) a blend of the polymer of a polymer of methacrylonitrile prepared by emulsion polymerization in the presence of a cationic emulsifier or the copolymer of (a) with a photospeed-enhancing amount less than 5 weight percent of a copolymer of vinyl acetate and vinyl chloride which would be incompatible with said polymer or copolymer of methacrylonitrile; and

an effective gas-producing amount of a photosensitive solid agent substantially uniformly dispersed within said coating, which agent is capable of decomposing to produce nitrogen gas upon exposure to light.

\* \* \* \* \*

25

30

35

40

45

50

55

60

65